

June 16, 1942.

H. A. LIEBHAFSKY

HEAT TREATING PROCESS

2,286,745

Filed Jan. 16, 1942



Inventor:  
Herman A. Liebhafsky,  
by Harry E. Dunham  
His Attorney.

## UNITED STATES PATENT OFFICE

2,286,745

## HEAT TREATING PROCESS

Herman A. Liebhafsky, Schenectady, N. Y., assignor to General Electric Company, a corporation of New York

Application January 16, 1942, Serial No. 427,032

5 Claims. (Cl. 148—13.2)

This invention relates to a process of heat treating metal articles. It is particularly concerned with the heat treatment of metal, specifically copper or copper alloy, strips or wires by immersion thereof in a molten metal bath.

The heat treatment of metal articles is often carried out by immersing the articles in molten metal baths, particularly lead or lead alloy baths, held at heat treating temperatures. This method requires simple and inexpensive apparatus and is advantageous also because of the rapid transfer of heat from the bath to the articles being treated. However, as far as I am aware, such baths have never been successfully used in commercial heat treatment of metals such as copper and its alloys which are easily wet by the molten metal or its oxides. When a copper wire, clean or oxidized, is passed through molten lead, the wire is quickly coated with lead or its impurities such as lead oxide making the annealed wire unfit for many applications, particularly the application of varnishes such as organic enamels.

An object of the present invention is to provide a new and improved process for heat treating metal articles in a bath of molten metal. Another object of the invention is to provide a method of preventing contamination of the heat treated article by the molten metal heat treating bath. A further object of the invention is to provide the metal articles, prior to heat treatment, with a protective coating capable of effectively preventing direct contact thereof with the molten metal and of being easily removed therefrom subsequent to the heat treating step.

The above objects are attained in accordance with my invention by coating the metal articles with a soluble alkali metal silicate before they are passed through a treating bath of molten metal over which a non-oxidizing atmosphere is maintained. After the articles have cooled to non-oxidizing temperatures, the protective silicate coating is removed by subjecting the wire to suitable acid and/or water washes.

My continuous process of heat treating metal articles, specifically copper strips or wires, by means of a molten metal bath may be better understood by reference to the accompanying drawing showing somewhat schematically a vertical, cross-sectional view of one type of apparatus that may be employed in the practice of my invention. For purposes of illustration the annealing of a copper wire will be considered.

With reference to the drawing, the wire 1 coming from a pay-off reel (not shown) passes over a pulley 2 and downwardly into intimate contact

with an applicator 3 of felt or similar material moistened with a suitable dilute aqueous silicate solution. Additional silicate solution is continuously or intermittently supplied to the applicator from conduit 4 which is connected through valve 5 with a reservoir 6 containing a supply of solution. The silicate solution may comprise any soluble silicate, such as the commercial sodium or potassium silicates, preferably those silicates having low alkali contents. For example, an entirely satisfactory coating has been obtained using a commercial sodium silicate solution containing 6.3 per cent  $\text{Na}_2\text{O}$ , 24.6 per cent  $\text{SiO}_2$  and 69.1 per cent water made up into a dilute solution by the addition of 7 parts water to 1 part of the silicate solution.

After being coated with a thin film of the silicate by contact with the applicator, the wire passes through an oven 7 where excess moisture 10 is removed from the silicate film before the coated wire enters the heat treating chamber 8 containing a molten metal heat treating bath 9. The drier 7 is not indispensable and may be omitted when sufficient drying of the soluble silicate film can be obtained by contact of the wire with the heated atmosphere above the molten metal bath.

For purposes of illustration I have shown the heat treating chamber 8 as comprising a flanged 30 container 10 provided with a flanged cover 11 in relatively gas-tight contact therewith. Suitable tubular passageways 12 and 13 are provided in the top of the cover 11 through which the wire enters and leaves the heat treating bath. A suitable reducing gas, preferably hydrogen, is introduced into the heat treating chamber through inlet pipe 14 in the side of cover 11 and prevents oxidation of the molten metal which is heated by means of gas burners 15 beneath container 10. 40 Excess gas escapes through wire passageways 12 and 13. The wire 1 after entering the heat treating chamber 8, passes beneath sheave 16, partially or wholly immersed in the molten lead or lead alloy bath 9, and is heated by the bath to annealing or other desired heat treating temperatures. From the heat treating bath the wire passes over suitable pulleys 17 and 18 and beneath a sheave 19 immersed in acid bath 20. The silicate film adequately protects the hot wire from oxidation by the atmosphere during its travel from the molten bath to the acid bath. 50 As the heat treating bath is ordinarily held at a temperature of about 400° C. for annealing copper per wire, unprotected copper heated to such tem-

peratures would be quickly oxidized by contact with air.

The acid bath preferably comprises a dilute (2 per cent) solution of hydrofluoric acid capable of completely removing the silicate film as well as any dirt or oxides picked up by the coated wire from the molten bath. Except for these contaminations, all of the protective silicate coating can be removed by a hot or cold water bath. However, a heat treated wire which has been washed only with water will be found to have a few widely separated "dirt" spots marring its otherwise bright, clean surface. These spots are readily removed by the dilute hydrofluoric acid bath indicating that the spots are not on the wire but on the silicate film which is preferentially attacked by the dilute acid.

The clean, acid-washed wire passes over pulley 21 and under sheave 22 immersed in a water bath 23 where the wire is freed of any traces of acid collected during immersion in the acid bath. From the water bath the clean wire passes over pulley 24 to a take-up reel after first being freed of water by air or oven drying. Air drying is sufficient if water bath 23 is maintained at or near its boiling point.

Copper wire annealed or heat treated by the above process can be coated, without further processing, with any of the usual wire enamels.

Although I have described my invention with particular reference to the annealing of copper wire, it is not restricted thereto but is generally applicable to the heat treatment of any metal article that can be dipped, sprayed, or otherwise provided with a protective silicate film prior to immersion in the molten metal bath.

What I claim as new and desire to secure by Letters Patent of the United States is:

1. A process for heat treating metal articles which comprises coating said articles with an alkali silicate, immersing the coated articles in a fused lead bath at heat treating temperatures and washing said heat treated articles to remove the alkali silicate coating.
2. In the process of heat treating metal articles by immersion thereof in a molten metal bath, the step which comprises coating said articles prior to heat treatment with a soluble alkali silicate.
3. In the process of heat treating metal articles by immersion thereof in a molten lead bath, the step which comprises coating said articles prior to immersion with a soluble silicate capable of protecting said wire from contamination by the molten lead.
4. A process of heat treating metal wire which comprises coating said wire with a layer of soluble alkali silicate, passing said coated wire through a molten lead bath while maintaining a reducing atmosphere above said bath, cooling said wire and thereafter washing said wire to remove the alkali silicate coating.
5. A process for heat treating copper wire which comprises coating said wire with soluble silicate, passing said coated wire through a heat treating bath of molten lead while maintaining a hydrogen atmosphere over said bath, passing said wire through a dilute hydrofluoric acid bath to dissolve the silicate coating and thereafter washing said wire to remove the acid adhering thereto.

HERMAN A. LIEBHAFSKY.